

April 9, 1935.

J. S. POU

1,997,153

MANUFACTURE OF ALPHA CELLULOSE

Filed Feb. 23, 1934



Inventor  
José Sala Pou.

By William C. Linton.  
Attorney.

This is a continuation of my application filed on January 23, 1934, Serial No. 500,320, and claims the benefit of the filing date of that application.

# UNITED STATES PATENT OFFICE

1,997,153

## MANUFACTURE OF ALPHA CELLULOSE

Jose Sala Pou, Barcelona, Spain

Application February 23, 1934, Serial No. 712,628  
In Spain October 21, 1933

3 Claims. (Cl. 92—13)

I have filed an application in Spain on the 21st October, 1933.

The present invention relates to the manufacture of alpha cellulose, and more particularly to a process for manufacturing this product from bamboo canes in a form suitable for the production of cellulose esters as substitutes for cotton pulp and its derivatives.

The plants of the order Graminaceæ, species 10 of bamboos, have fibres possessing special characteristics, a fact which has already been known to paper manufacturers; but the said fibres have not hitherto been used for the manufacture of super-alpha celluloses capable of competing in 15 the market with the super-alpha celluloses derived from cotton.

The nature of the plants, which are different in their constitution from wood, leads to the assumption of the possibility of the formation of a cellulose compound which being less lignified, may give characteristics more similar to the polymerization of the cotton molecule. On the other hand, the greater percentage of lignine which the plants contain as compared to the other 25 plants of the order Graminaceæ, allows also of the bamboos producing a cellulose in the form of filaments having fibro-vascular fascicles of a greater length than those of the other plants of the order.

30 The applicant has discovered a process which makes it possible to eliminate the peptins which form the non-cellulosic group, as distinct from the lignines which enter into the composition of the plant.

35 These substances which have the property of combining with the lignines at the high reaction temperatures which are reached in the classic bisulphite, soda and sulphide processes, give compounds which strongly dye the fibres with a product which gives a dark brown reaction with bleaching chlorine and which can be with difficulty eliminated by the latter unless the chlorine is used in proportions which always produce considerable oxidation of the fibres. Moreover, the 40 45 peptins can be easily rendered soluble by alkaline hydrates at temperatures in the neighbourhood of 110 degrees.

In view of the simplicity with which the peptins are eliminated the idea has been conceived 50 to use in place of a continuous process, a fractional process which at a first boiling at a pressure of 0.5 atmosphere in an alkaline lye containing 1.5 per cent of the corresponding alkali, in the proportion of 1:5 between the weight of the 55 material treated and the weight of the bath, elim-

inates the peptins. This quantity of hydrate is sufficient for converting them into the form of a soluble salt which remains in solution. The combination of sugars, starches and peptins formed, owing to the excess of alkali which remains in the bath without reacting, cannot be abstracted, as otherwise it would be precipitated and would stain the cellulose fibre to such an extent that it would be difficult to clean it.

The alkaline hydrates, even at the low temperatures at which the operation is carried out, always exert a hydrolyzing effect on the hemi-celluloses which accompany the alpha cellulose, and the oxidizing molecules of the hydrates always exercise some hydrolytic action also on the alpha 1 celluloses. For that reason it has been considered advisable to introduce in the first stage a reducing element such as an alkaline sulphite or sulphites, which combining with oxygen, prevents the said hydrolyzing effect and leaves the elimination of the lignine and of the semi-celluloses to the second stage of the process, so that the first stage thereof serves only for the elimination of the above-mentioned substances.

The combined action of the alkaline hydrates 2 and of the alkaline sulphites must take place at the temperature and pressure indicated and within a period of time of two to four hours. As soon as this first stage of the operation is completed, the pulp is washed first with hot water and then 3 two or three times with cold water. Into the autoclave in which the operation is carried out, a new lye which contains per litre 45 grammes of alkaline hydrate, 20 grammes of sulphide of sodium and 5 grammes of sulphite of sodium is 3 then introduced.

The first object aimed at by the use of this lye is to avoid the effects of hydrolyzation which have been provided for in the first stage. Sodium sulphide and sulphite are intended to attain this 4 object. For the same purpose the lye in the form of sodium sulphide and caustic soda, could also be combined in any proportion which may be considered suitable for combining the said products 4 with the lignine.

The highly beneficial reducing effect of the sodium sulphide for obtaining super-alphas may be assumed to be represented by the following equation:



This reaction, which, as indicated is reversible, is a hydrolysis which gives sodium sulphohydrate, and this product forms the reducing atmosphere 5

which prevents the effect of oxidation on the alpha cellulose.

The acid contents of the lignine or the lignitic acids are neutralized by the alkaline hydrate or by 5 the hydrolysis of the Na<sub>2</sub>S to NaOH, giving soluble soda compounds.

The NaHS combines with alcohols (to form mercaptans) and with phenols, the result of the reaction being by weight, with regard to the sulphide, as follows:

|                                                | Per cent |
|------------------------------------------------|----------|
| Combined with the lignine after the hydrolysis | 51.8     |
| Retained by volatile organic substances        | 15.0     |
| 15 Remaining unaltered as Na <sub>2</sub> S    | 15.8     |
| Eliminated in the form of sulphate             | 17.8     |

This oxidation of sulphide in order to pass to sulphate takes place at the expense of active oxygen which would have produced oxidizing action on the alpha celluloses.

The temperatures applied for the elimination of the lignine start at 140 degrees C., but in some kinds of old bamboos, that is to say, bamboos which are in the advanced period of lignification, or in the bamboos which grow in shallow soils which prevent the roots of the plant from penetrating deeply into the earth and where the rainy periods are very rare or the rain is scarce between the stage of first growth of the stem and the stage of second growth in which latter the branches and the leaves appear, as a result of which there is a lack of moisture in the roots and therefore in the plant, with the consequent quick drying up of the starches in the fundamental parenchyma of the plant, on the said alimentary substances being eliminated for the normal development of the cellulose until its maximum uniform growth is reached, there takes place a premature ageing, so that a premature kind of very much condensed lignine is produced which strongly envelops the fibres in the ligneous fibro-vascular sheafs or faggots, and which is difficult to eliminate by the industrial processes for the elimination of the said product, and in such cases it is necessary to use high temperatures of 170 degrees C. which produce on the other hand a serious hydrolysis of the alpha cellulose.

In spite of the reducing atmosphere which the sulphide produces, it has been found difficult to avoid these actions, and in order to avoid also such high temperatures, and it has been attempted to find some solvent for the lignine. A suitable solvent has been finally found among the ethers of the phenols. As an example of this solvent, may be used guayacol, that is to say monomethyl ether of the phenol which is found in ample quantities in beech tar, and in its corresponding creosote oil. This substance greatly assists the effect of the lye since lignine is a resin and as such on being attacked by soda, becomes viscous and forms a film which envelops the fibro-vascular bundles which offer a colloidal resistance to penetration by new portions, which has to be overcome by making it more fluid by an increase of temperature and pressure, with the drawback which this involves, viz; the hydrolysis of the cellulose. The guayacol quickly dissolves the coating of lignine gelatinized by the hydrate and allows new portions of the lye to attack rapidly new zones of lignine. Owing to the action of the guayacol it is possible, even in cases where old bamboos or bamboos grown in bad conditions are used, to do without varying the times and the pressures required for the operation, and in these

conditions with one hour at 156 degrees C. and the corresponding pressure, and with two or three hours at 140 degrees C. and the corresponding pressure, it is possible to reduce these plants, which with the old treatment would require a pressure of 8 atmospheres.

After the completion of the boiling, a further washing operation with hot water is carried out. When guayacol has been used, the first water is emulsified with a benzol in the proportion to the quantity of the guayacol used, plus 50% by weight of this body. After twice washing with hot water, the product is washed two or three times with cold water, and thereupon bleached with a hypochlorite solution of one half to one degree Bé. This cellulose thus obtained is washed and submitted to the action of a HF bath of half percent. In this way the remains of the silica are eliminated, and the residue of ashes can be reduced to 0.3%. After this bath, the product is washed in plenty of water, and the bleached cellulose is subjected to the action of a solution of bisulphite of soda of 2° Bé. at a temperature which may vary between 60 degrees C. at atmospheric pressure and 120 degrees C. at a pressure of one atmosphere. This operation eliminates the quantities of oxi- and hydrocellulose, and the rest of the lignine that may still be left. After this bath, the cellulose is washed in plenty of water and may be submitted if desired to the action of a solution of peroxide of sodium or of peroxide of hydrogen for the purpose of improving its whiteness.

The cellulose obtained by this process from the bamboos has exceptional characteristics which are in no way inferior to the characteristics of cotton.

For carrying out the reactions and operations above set forth it is preferred to employ an installation comprising a combination of elements, by means of which the whole process according to the invention can be carried out automatically from the commencement up to the delivery of the cellulose without the necessity for manual operations.

A preferred constructional arrangement of such an installation is illustrated by way of example in the only figure of the accompanying drawing.

Referring to the drawing:

The cut bamboos after having been left to dry in the field for a period of forty days, are exposed to the action of running water, either in a river or in suitable pools for a period of time which varies from 7 to 15 days.

The bamboos prepared in this way are introduced into a grinding mill 1 constituted by four pairs of cylinders or rollers, two of which are provided with grooves or flutes, and these two rollers owing to the action of hydraulic pressure applied to them, flatten and break the joints or knots of the bamboos. The other two pairs of rollers are provided with teeth arranged in zig-zag shape and are also subjected to strong hydraulic pressure, their object being to cut the bamboos. This operation is of the greatest importance, inasmuch as, the uniformity of the boiling depends on the elimination of the air from the perforated vessels, since the said air may cause the mass to float in the boiling lye, which would retard by at least one hour the time of immersion.

The bamboo stems having been cut to portions of about one square centimetre section and completely disintegrated, drop into a pit which is lo-

- cated in front of buckets 2 which lift the cut stems up to the hopper 3. The said hopper is so dimensioned that its capacity is the same as that of the autoclave 4 with which it is associated.
- 5 The said autoclave receives the new lye which is supplied from 18, and which has been mixed in a well 19 provided with an agitator, with the regenerated lyes coming from the tank 26.
- As soon as the cut bamboo and the lye have 10 been introduced in the said manner into the autoclave, steam is admitted from a steam generator 20 the said steam being used for indirect heating so as to avoid any dilution of the bath. This point, though it is not of much importance in 15 the production of cellulose intended for the manufacture of paper, is important in the case of those super-alpha celluloses in which variations to the extent of one tenth percent in the lye are liable to produce variations of more than 20 two percent in the contents of the alpha. At the proper moment, the top valve of the apparatus is opened, and a circulating pump with which it is provided, is started, for the purpose of enabling the air contained in the mass consisting 25 of lye and bamboo to be expelled. This operation is of great importance as it avoids the oxidation of the cellulose by the oxygen of the air. As soon as this operation is finished, the temperature is raised until the pressure previously 30 stated is reached and is maintained during the period of time also stated, whereupon the lye is discharged through a valve and sent for recovery or recuperation. The mass contained in the autoclave, is thereupon washed once with 35 hot water and three times with cold water.
- This first stage of boiling of the bamboo being finished, the lye by means of which the second operation or stage is carried out, is introduced into the autoclave, the same precautions 40 being taken with regard to the air as were adopted in the previous operation, and a continuous circulation being kept up during the boiling operation by means of the pump already referred to. As soon as the operation is finished and after 45 the washing operations which follow those with emulsified benzol, the lye is returned to the well 5 from which it passes together with the first two washing waters, to a tank 21 serving for the reception of the lyes which are to be 50 treated for recovery or recuperation.
- The lyes from the tank 21 are conveyed to a multiple action evaporator 22 which is fed with the steam coming from the steam generator 20 and afterwards pass to the rotary oven 23 in 55 which they are calcined and from the latter pass to the pit 24 from which an Archimedean screw raises them to the caustifying vessels 25 from which they pass to settling tanks 26.
- As soon as the lyes have been conveyed to the 60 recovery units, the cellulose is returned to the well 5 in which it is diluted with water and washed therewith, being stirred for the purpose by a powerful agitating device. The pulp which is thus formed, is conveyed by means of a pump 65 to a "thickener" or concentrator 6 which in its turn after having eliminated the water, delivers the pulp to a disintegrator-defibrator of the kind known under the name of "cone breaker". This disintegrator is sufficient for the purpose in- 70 as much as the material to be treated is thoroughly boiled pulp which does not normally contain any knots (since it has been ground in the mill 1); but in cases in which, owing to some defect in the grinding mill, the knots of the bamboos 75 had not already been sufficiently ground, it would
- be necessary to interpose between the well 5 and the concentrator 6, one or more rotary purifiers working with one millimetre pitch.
- On being discharged from the cone breaker, the pulp is introduced into one or more washing and bleaching vats or machines 8 to which is supplied a solution of sodium hypochlorites supplied from decanting devices 30. From the said washing and bleaching machine or machines 8 the cellulose passes to a vat 9 where it is treated 10 with hydrofluoric acid of the above-mentioned concentration. This vat is lined inside with a plastic material having for its basis rubber, in order to render it proof against the action of the acid which comes from a supply unit 29.
- The cellulose passes from the vat 9 to a vat 10 in which it is washed with plenty of water until the last traces of the acid are removed and from the said vat the cellulose passes to a concentrator 11 from which it is here conveyed by a 15 pump into an autoclave 12.
- The cellulose is introduced into the autoclave 12 through the bottom part of the latter and is forced to circulate through several inclined planes arranged in the interior of the said autoclave, and at the proper time the corresponding solution of sodium sulphite is introduced. The bath is thereupon heated by means of steam coming from the steam generator 20 and passing through a closed coil arranged at the bottom of 20 the apparatus. In these conditions, the pressure rises to one atmosphere, and the pulp is extracted from the upper part of the autoclave by a pump provided with a special pressure-relief device. On its discharge from the said pump, the 25 pulp passes into a vat 13 in which it is thoroughly washed. The sulphite used in the last named lye is supplied from a unit 27.
- The pulp contained in the vat 13, after having been treated in the latter, passes to the vat 14 30 where it is treated with a solution which is prepared in a unit 28 and which is composed of sodium peroxides or hydrogen peroxides, and on leaving the vat 14, the pulp passes through a long sand-removing device 15, from the latter 35 to a centrifugal purifier 15 and finally to a pulp press 17.
- The pulp thus obtained which contains from 40 97 to 98% of alpha cellulose is of a magnificent white colour, and its fibres are 7 to 8 millimetres 45 long. This super-alpha cellulose with such exceptional characteristics, extracted from bamboos, is obtained in a proportion of 35 to 40% of the dry plant and is more particularly suitable 50 for the esterification as well as for the manufacture of papers, particularly of papers for documents, ledgers and bank notes. Moreover in view of the exceptional absorption capacity 55 which this fibre possesses, it can be used in place of cotton for the hygienic and sanitary purposes 60 for which the latter is employed.
- The product obtained by the process hereinbefore described, has the following characteristics:
- |                                                                                      |            |    |
|--------------------------------------------------------------------------------------|------------|----|
| Alpha cellulose                                                                      | 96-98%     | 65 |
| Beta cellulose                                                                       | 1-1.5%     |    |
| Gamma cellulose                                                                      | 0.5%       |    |
| Lignine                                                                              | 0.5%       |    |
| Copper index                                                                         | 0.6-1.5%   |    |
| Resins etc.                                                                          | 0.07       | 70 |
| Average length of fibre                                                              | 8 mm.      |    |
| Herzberg colouration                                                                 | Purple red |    |
| Ash residue                                                                          | 0.3%       |    |
| Viscosity equal to that of pure normal cotton in a cupro-ammoniacal solution of 0.5% |            | 75 |

The process described may vary as regards the apparatus and machines employed for carrying it into practical effect and the arrangement of the latter and it will be understood that the 5 installation fully described and diagrammatically illustrated in the accompanying drawing is merely given as an example of one of the possible methods of carrying the said process into practical effect. The purpose for which the 10 product obtained by the said process is intended, as well as the form of its presentation for the subsequent use may also vary and generally the process, installation and product may be modified in various ways without departing from the 15 scope of the invention.

I claim:

1. A process for the manufacture of alpha cellulose from bamboos, comprising in steps: drying cut bamboo in the open air; exposing the 20 cut and dried bamboo to the action of running water; grinding said bamboo to form a kind of tow; boiling said tow in an autoclave with a lye composed of alkaline hydrates and a reducing agent at a pressure of .5 to 1 atmosphere; washing 25 said tow in the autoclave first with hot water and then with cold water; subjecting the bamboo pulp thus produced in the same autoclave to the action of a second lye containing alkaline hydrate, sodium sulphide, sodium sulphite and 30 guayacol for one hour at 156° C. and 4.8 atmospheres pressure, and for a few hours at 143° C. and 3 atmospheres pressure; washing the pulp in the autoclave first with water emulsified with benzol and then three times with cold water; dis- 35 charging the pulp into a tank fitted with an agitator and diluting it with water; passing the pulp through a thickener and then through a disintegrator-defibrator; subjecting the pulp to the oxidizing action of sodium hypochlorite lye, 40 washing it in plenty of water and subjecting it then to the action of a bath of hydrofluoric acid and again washing with ample water; passing the pulp through a thickener and then into an autoclave in which it is mixed with a suitable quantity of sodium sulphite at 60° C. and 2 atmospheres pressure and then washed; and bleaching 45 the pulp with hydrogen peroxide or sodium peroxide, washing it, and converting it into solid form.
2. A process for the manufacture of alpha cellulose from bamboos, comprising in steps: drying cut bamboo in the open air; exposing the cut and dried bamboo to the action of running water; grinding said bamboo to form a kind of tow; boiling 50 said tow in an autoclave with a lye composed of alkaline hydrates and a reducing agent at a pressure of .5 to 1 atmosphere; washing said tow in the autoclave first with hot water and then with cold water; subjecting the bamboo pulp thus produced in the same autoclave to the action of a second lye containing alkaline hydrate, sodium sulphide, sodium sulphite and guayacol for one 55 hour at 156° C. and 4.8 atmospheres pressure, and for a few hours at 143° C. and 3 atmospheres pressure; washing the pulp in the autoclave first with water emulsified with benzol and then three times with cold water; discharging the pulp into a 60 tank fitted with an agitator and diluting it with water, thereby washing it again and then passing it through a disintegrator-defibrator; subjecting the pulp to the oxidizing action of sodium hypochlorite lye, washing it in plenty of water and then subjecting it to the action of a bath of hydrofluoric acid and again washing with ample water; passing the pulp through a thickener and then into an autoclave in which it is mixed with a suitable quantity of sodium sulphite at 60° C. and 2 atmospheres pressure and then washed; bleaching the pulp with hydrogen peroxide or sodium peroxide, washing it, and converting it into the usual known solid form.

tank fitted with an agitator and diluting it with water; passing the pulp through a rotary purifier having a pitch of 1 millimetre for removing any bamboo knots which have still been left unground during the previous mechanical action to which the pulp has been submitted; passing the pulp through a thickener and then through a disintegrator-defibrator; subjecting the pulp to the oxidizing action of sodium hypochlorite lye, washing it in plenty of water and subjecting it then to the action of a bath of hydrofluoric acid and again washing with ample water; passing the pulp through a thickener and then into an autoclave in which it is mixed with a suitable quantity of sodium sulphite at 60° C. and 2 atmospheres pressure and then washed; and bleaching the pulp with hydrogen peroxide or sodium peroxide, washing it, and converting it into solid form:

3. A process for the manufacture of alpha cellulose from bamboos, in a form suitable for conversion to cellulose esters as substitutes for cotton pulps and derivatives comprising in steps: drying the cut bamboo in the field in the open air for forty days; exposing the cut and dried bamboo to the action of running water in a river for from 7 to 15 days; grinding said bamboo to form a kind of tow; boiling said tow in an autoclave for a period of 2 to 3 hours with a circulating lye, the ratio between the amount of the 30 tow and the lye being 1:5, and the lye being composed of alkaline hydrates together with 1.5 to 2 percent of a reducing element, the boiling operation taking place at a pressure of .5 to 1 atmosphere and the temperature corresponding thereto; washing said tow in the same autoclave first with hot water and then three times with cold water; subjecting the bamboo pulp thus produced in the same autoclave to the action of a second lye containing per litre 45 grammes of 40 alkaline hydrate, 20 grammes of sodium sulphide and 5 grammes of sodium sulphite together with a suitable quantity of guayacol, the lye being caused to circulate through the bamboo pulp for 1 hour at 156° C. and 4.8 atmospheres pressure, and then for 2 to 3 hours at 143° C. and 3 atmospheres pressure; washing the pulp in the autoclave first with water emulsified with benzol in the proportion of one-and-a-half times the weight of the guayacol and then three times with cold water; discharging the pulp into a 50 tank fitted with an agitator and diluting it with water, thereby washing it again and then passing it through a disintegrator-defibrator; subjecting the pulp to the oxidizing action of sodium hypochlorite lye, washing it in plenty of water and then subjecting it to the action of a bath of hydrofluoric acid and again washing with ample water; passing the pulp through a thickener and then into an autoclave in which it is mixed with a suitable quantity of sodium sulphite at 60° C. and 2 atmospheres pressure and then washed; bleaching the pulp with hydrogen peroxide or sodium peroxide, washing it, and converting it into the usual known solid form.

JOSE SALA POU.